

Nov. 11, 1941.

W. T. MONTAGUE

**2,262,618**

## NONSLIP BRICK

Filed Feb. 14, 1939



Fig. 1

FIG. 4



Fig. 2

Fig. 3



Inventor  
WILLIAM MONTAGUE

Inventor

By George Compton Jr.

Attorney

## UNITED STATES PATENT OFFICE

2,262,618

## NONSLIP BRICK

Wallace T. Montague, Worcester, Mass., assignor  
to Norton Company, Worcester, Mass., a corporation of Massachusetts

Application February 14, 1939, Serial No. 256,331

## 3 Claims. (Cl. 72—36)

The invention relates to non-slip bricks and tiles.

One object of the invention is to provide an apparatus for manufacturing non-slip tile and bricks by the use of which they can be manufactured economically. Another object of the invention is to provide a packing house brick which will wear indefinitely and prevent accidents. Another object of the invention is to provide an extrusion method for the forming of bricks with abrasive in one surface only. Another object of the invention is to form a composite brick structure in a single operation. Another object of the invention is to provide an apparatus and method for manufacturing bricks having a layer of abrasive material in accordance with which the ultimate product is integral and not liable to spalling, chipping or separation. Other objects will be in part obvious or in part pointed out hereinafter.

The invention accordingly consists in the features of construction, combinations of elements, arrangements of parts, and in the several steps and relation and order of each of said steps to one or more of the others thereof, all as will be illustratively described herein, and the scope of the application of which will be indicated in the following claims.

In the accompanying drawing illustrating one of many possible embodiments of the mechanical features of this invention,

Figure 1 is a vertical sectional view of apparatus for forming "green" bricks;

Figure 2 is a plan view of the apparatus; and

Figure 3 is a sectional view taken along the line 3—3 of Figure 1.

Figure 4 is a perspective view of a brick according to the invention.

As conducive to a clearer understanding of the present invention, it is noted that in packing houses there is a quick accumulation on the floor of waste matter, blood and the like. This has to be cleaned off at regular intervals or it decays and putrefies which would not be healthful and would affect the meat. In order to clear the floors, it has been customary to use hot water or live steam. This would quickly deteriorate any wooden floor and, therefore, brick floors have been provided. Because of reasons of economy, the brick used has been of a cheap variety, for example made of red clay vitrified at a low temperature. Such bricks have not been entirely satisfactory for the reason that they are quite slippery under packing house conditions and,

furthermore, they wear fairly rapidly, thus requiring replacement.

Various types of non-slip tiles have been provided in the past but methods of manufacture heretofore known have been too expensive for the manufacture of packing house bricks to compete with the ordinary product. By my invention I provide a packing house brick having a non-slip surface and an apparatus and method of manufacture thereof permitting it to be manufactured relatively cheaply so that although somewhat more expensive than the ordinary plain brick, this will be in part at least compensated for by the increased life of my product, whereas the non-slip nature thereof is a definite advantage.

Referring now to Figure 1, I provide a machine comprising legs 10 supporting a table 11 upon which is mounted a hollow cylinder 12. Above the hollow cylinder 12 and communicating with it by means of an orifice 13 is a hopper 14. In the hollow cylinder 12 is a feed screw 15 substantially completely filling the inside of the cylinder 12 and mounted on a small diameter shaft 16 so that material fed into the hopper 14 will be moved to the right in the cylinder 12. The shaft 16 is supported at the right-hand end in a journal 17 integral with a grid 18 which stops the rotation of the material. The shaft 16 is supported at the left-hand end in a journal 20 formed integral with a cylinder head 21. On the left-hand end of the shaft 16 is a bevel gear 22 meshing with a bevel gear 23 on a vertical shaft 24. The shaft 24 is supported in a vertical thrust bearing 25 formed in a bracket 26 fastened to a pair of legs 10. Near the bottom of the shaft 24 is a bevel gear 27 meshing with a bevel gear 28 on the left-hand end of a drive shaft 29. A pulley 30 on the drive shaft 29 is connected by a belt 31 to a pulley 32 on the armature shaft 33 of an electric motor 34. Thus the screw 15 is rotated and in such a direction that material fed into the hopper 14 will be moved to the right in the cylinder 12.

Integrally formed with the cylinder 12 is another cylinder 35 whose axis intersects that of the cylinder 12 but is inclined thereto at an angle of about 45°, although the angular relationship is not critical. In this cylinder 35 is a feed screw 36 mounted on a shaft 37 which is journaled in a journal 38 formed integral with a grid 39 to stop rotation of the material. The shaft 37 is journaled at its upper end in a journal portion 40 formed in a hopper 41 having a bottom opening 42 communicating with the upper part of the

cylinder 35. On the upper end of the shaft 37 is a bevel gear 43 meshing with a crown gear 44 on the end of a shaft 45 journalled in a journal 46 attached to brackets 47 extending from the hopper 41 to a bracket 48 (see Figure 2) supported by brackets 49 fastened to the table 11. On the under side of the bracket 48 is a journal 50 also supporting the shaft 45, on the left-hand end of which is a bevel gear 51 meshing with a bevel gear 52 on the upper end of the shaft 24.

Still referring to Figure 1, a baffle plate 53, which may be curved and of the same radius as the cylinder 12, intercepts the opening at the bottom of the cylinder 35 and forms a continuation of the cylinder 12. A continuation 12a of the cylinder 12 receives material inserted in the hoppers 14 and 41 where the materials merge. An extrusion nozzle 55 closes the cylindrical end of the cylindrical extension 12a and is bolted to it as shown. In cross section the shape of the nozzle 55 gradually changes from a circle to a rectangle and the delivery opening 56 is trapezoidal in shape.

I provide ceramic mixtures of suitable brick clay and brick clay mixed with abrasive grains. The brick clay may be the ordinary red brick clay now used for the manufacture of packing house bricks. A plain mixture of red brick clay is constantly fed by the operator into the hopper 14. A mixture of this clay and abrasive grains is constantly fed by the operator into the hopper 41. Preferably the mixture in the hopper 41 consists of the order of 25% abrasive by volume and 75% clay by volume. The abrasive may be of any suitable variety, but I prefer to use electric furnace fused alumina in grit sizes from 20 mesh to 8 mesh and even coarser. A preferred grit size is 8 mesh grit size. These sizes define abrasive grains which will just pass through a screen having that many meshes to the linear inch in pick and sley. Other abrasives, however, can readily be used, especially such as silicon carbide and flint (quartz), and the invention is not limited to any particular mesh size of the abrasive used.

It will now be seen that the extrusion apparatus forces the ordinary clay mixture through the cylinder 12 and forces the mixture of clay and abrasive down the cylinder 35 where the two streams merge, the grids 18 and 39 stopping the rotation of the mixture and causing the abrasive mixture to assume a position on top of the plain mixture. Thus through the trapezoidal opening 56 is forced a quantity of ordinary clay on the bottom and a mixture of clay and abrasive on the top. It is not represented that the line of division is at all times perfectly straight and even but this is not a matter of great consequence.

The gear ratios of the driving mechanism cause the screw 15 to be driven about four times as fast as the screw 36 which will feed four times as much ordinary clay as mixture of clay and abrasive and permit the application of a layer of clay and abrasive on the top of the extrusion mass to be approximately one quarter the depth thereof.

The opening 56 has been referred to as trapezoidal and it will be noted that it is but slightly removed from a rectangle. In fact, the lateral edges can be at right angles to the bottom line near the bottom line and then form an obtuse angle with the top line. The reason for slightly altering the otherwise rectangular shape of the orifice 56 is that during firing, the mixture of clay and abrasive expands more than the portion consisting simply of clay so that to produce

a truly rectangular parallelepipedal brick, it is desirable to shape the nozzle 56 as indicated.

The formed clay body with abrasive on the top emerges from the orifice 56 in a steady stream trapezoidal in cross section. This steady stream of extruded clay and abrasive should be cut off into suitable lengths to form "green" bricks. If desired, this may be done by hand and the top of the table 11 may be provided with a scale. If desired, I provide a second long table 60a on to which the material may move as it passes off the table 11. I prefer to provide some mechanical means for cutting off the extruded clay, such as a flying shear or the apparatus which will now be described.

Referring now to Figure 1, on the under side of the table 11 and depending therefrom are a pair of journals 60 and 61 for the shaft 29. At the right-hand end of the shaft 29 near the journal 61 is a crowned gear 62 which meshes with a gear 63. Referring now to Figures 1 and 2, the gear 63 is on a shaft 64 to which is fastened a pulley 65 connected by a belt 66 to a pulley 67 on the end of a transverse shaft 68 which extends over the table 11. The shaft 68 may be journalled in suitable journal brackets 69 and 70. Fastened to the shaft 68 are a pair of spiders 71, the arms 72 of which have extending between them wires 73. As the machine is operated, the spiders 71 rotate, carrying the wires 73 downward, which cut off the extruded clay nearly in a plane perpendicular to the propagation thereof. Each brick can be quickly trimmed off with a trowel by the man who places them in a kiln to make the end surfaces normal to the top and bottom surfaces.

The "green" bricks are now taken to a suitable ceramic kiln and vitrified at temperatures commonly employed for firing packing house bricks. Such temperatures are fairly low in the ceramic arts but I will not further describe vitrification of the bricks since that may be done in accordance with usual practice. By reason of the fact that the bricks started out trapezoidal in cross section, the expansion brings them approximately to rectangular parallelepipeds.

It has been mentioned that the abrasive is of the order of 25%. To obtain a substantial effect from the abrasive, it should constitute at least 10% of the volume of the surface portion. That is to say, the surface area which contains the abrasive should have on the surface at least 10% of abrasive material measured by volume. In making this measurement by volume, the vertical dimension should be taken as one abrasive grain deep. On the other hand, there should not be more than 40% abrasive in any part of the block because more than this amount may cause such differences in the vitrifying that the brick will be deformed or the abrasive portion may separate from the plain portion.

It will thus be seen that there has been provided by this invention apparatus, a method and an article in which the various objects hereinabove set forth together with many thoroughly practical advantages are successfully achieved. As various possible embodiments might be made of the mechanical features of the above invention and as the art herein described might be varied in various parts, all without departing from the scope of the invention, it is to be understood that all matter hereinbefore set forth or shown in the accompanying drawing is to be interpreted as illustrative and not in a limiting sense.

I claim:

1. A non-slip brick comprising a substantially rectangular portion of plain vitrified red brick clay and a substantially rectangular layer integral with said first portion and comprising vitrified red brick clay with not more than 40% and not less than 10% of discrete particles of abrasive included therein.
2. A brick made of vitrified red brick clay and having its surface modified by an inclusion of between 10 and 40% of fused alumina abrasive grains in the surface area measured by volume.
3. A brick consisting of vitrified red brick clay having a surface containing discrete particles of abrasive which brick, measured to a depth consisting of the vertical dimension of the average abrasive in the surface, has a volume percentage of between 10 and 40% abrasive, the remainder ordinary vitrified red brick clay, the majority of the brick being substantially free from abrasive and consisting of ordinary vitrified red brick clay, the brick being an integral whole.

WALLACE T. MONTAGUE.